

H. G. REIST & H. MAXWELL.  
INDUCTION MOTOR.  
APPLICATION FILED MAR. 31, 1915.

1,190,009.

Patented July 4, 1916.

Fig. 1.



Fig. 2.



Fig. 3.



Fig. 4.



Inventors:  
Henry G. Reist,  
Howard Maxwell,  
*Alvord, Davis*  
by  
Their Attorney

# UNITED STATES PATENT OFFICE.

HENRY G. REIST AND HOWARD MAXWELL, OF SCHENECTADY, NEW YORK, ASSIGNEES  
TO GENERAL ELECTRIC COMPANY, A CORPORATION OF NEW YORK.

## INDUCTION-MOTOR.

1,190,009.

Specification of Letters Patent.

Patented July 4, 1916.

Application filed March 31, 1915. Serial No. 18,256.

To all whom it may concern:

Be it known that we, HENRY G. REIST and HOWARD MAXWELL, citizens of the United States, residing at Schenectady, county of Schenectady, State of New York, have invented certain new and useful Improvements in Induction-Motors, of which the following is a specification.

Our invention relates to induction motors and particularly to a method of and apparatus for casting squirrel cages in the magnetic cores of such motors.

It has for its object a simple method of manufacture, which requires a very simple mold.

To this end, our invention consists in pouring molten metal into a mold surrounding the magnetic core of an induction motor and simultaneously rotating the mold and core at sufficient speed to drive the molten metal into the conductor receiving openings in the core by centrifugal force, and continuing the rotation until the poured metal has congealed. In this way, the molten metal is caused to flow very quickly through the openings in the core before it chills, and it also forces any air out of the openings in the core which tends to be trapped therein. The mold is preferably formed with recesses for forming end or short-circuiting rings for the conductor bars. In carrying out our method, inner cores for the end rings are dispensed with, which allows the end rings to shrink uniformly upon cooling and thus prevents them from cracking.

Our invention also consists in a mold for carrying out this method.

For a better understanding of our invention reference may be had to the following description taken in connection with the accompanying drawing, in which—

Figure 1 is a view partly in section of a mold and core embodying our invention and by means of which our new method has been carried out; Fig. 2 is a section on the line 2—2 of Fig. 1; Fig. 3 is a sectional view of a squirrel cage cast in position on the secondary core of an induction motor; and Fig. 4 is a fragmentary view, similar to Fig. 1, of a modification.

Referring to the drawing, 1 is a secondary magnetic core member of an induction motor, the outer periphery of which is cylindrical. This core member is provided with

substantially longitudinally extending, conductor receiving openings therethrough. These openings may be either open or closed slots. In Figs. 1 to 3 they are shown as open, that is, with a small opening extending from the slot to the periphery of the core member. The laminations forming the core member 1 may be clamped together between plates 15 by means of bolts 16. The mold for the squirrel cage comprises cylindrical portions extending beyond the ends 65 of the core and end flange portions 3 and 4. The cylindrical portions in Figs. 1 and 2 are shown as comprised in a member 5, which preferably embraces the outer periphery of the core member 1 and is shown as 70 being divided along lines substantially parallel to the axis of the core member into a plurality of parts 5'. The parts 5' of the member 5 may fit in grooves in the flange portions 3 and 4, bolts 6 being provided for 75 clamping the portions of the mold in place, that is, the flange portions to the member 1. The end flange portion 3 has an opening 7 through which molten metal is received, the molten metal being caused to flow by 80 centrifugal force through the conductor receiving openings in the core member 1 to form an end ring 8 between the flange portion 4, the member 5 and the end of the core, conductors 9 in the openings in the 85 core member 1, and an end ring 10 between the flange portion 3, member 5, and the core member 1.

The mold and the core member 1 are rotated as a unit in any suitable manner. We 90 have shown for this purpose a mandrel 11 fastened in the shaft receiving opening 12 in the core member, the mandrel 11 having mounted thereon a belt pulley 13, the whole being rotated by means of a belt 14. While 95 the core and mold are being rotated, sufficient metal is poured into the mold to form the end rings 8 and 10 and the conductors 9, the rotation of the mold and the core being continued until the poured metal has congealed. When the casing has cooled sufficiently, the mold is removed by withdrawing the bolts 6, then removing the end flange portions 3 and 4 and the parts 5' of the member 5. The mandrel 11 is also removed 100 as may be the clamping plates 15 and the bolts 16. These clamping plates hold the laminations forming the core member 1 to-

gether until the squirrel cage is cast in place. As the laminations forming the core member become hot near their periphery due to the heat absorbed from the molten metal, their outer portions are liable to expand and buckle unless some provision is made for allowing the portions of the laminations near the shaft receiving opening 12 to expand. In Fig. 2, we have shown the laminations slit from the ventilating ducts 19 to the shaft receiving opening along lines 18 for this purpose. Fig. 3 shows a core member with the squirrel cage cast in place, and the mold, mandrel, clamping plates 15 and bolts 16 removed. An ordinary shaft is then driven into the shaft receiving opening 12 and permanent clamping plates for clamping the laminations together are placed in position and held in place by means of bolts or rivets extending through holes 17.

In the modifications shown in Fig. 4 the core member 1' is provided with closed slots. The mold for casting the squirrel cage in this case comprises cylindrical portions 2' extending beyond the ends of the core member 1' and end flange portions 3'. Such cylindrical end flange portions are provided at each end of the core member, but those at the upper end only are shown. The end flange portion 3' is provided with an opening 7' through which molten metal is received for forming the cast parts of the squirrel cage. The portions of the mold are clamped in place by means of bolts 6'. A casting is made in the same way as that described in connection with Figs. 1 and 3.

We prefer to use aluminum for this casting as it may be molded at a low temperature and is light in weight, but any other suitable metal, such as copper, may be used.

We desire it to be understood that our invention is not limited to the particular arrangement shown and described, and we aim in the appended claims to cover all modifications which do not depart from the spirit and scope of our invention.

What we claim as new and desire to secure by Letters Patent of the United States, is:—

1. The process of forming an induction motor squirrel cage on a magnetic core having substantially longitudinally extending, conductor receiving openings therethrough which consists in pouring molten metal into a mold surrounding the core and simultaneously rotating said mold and core at sufficient speed to drive the molten metal into the conductor receiving openings by centrifugal force, and continuing such rotation until the poured metal has congealed.
2. The process of forming an induction motor squirrel cage on a magnetic core having substantially longitudinally extending, conductor receiving openings therethrough which consists in pouring molten metal into a mold surrounding the core and simultaneously

rotating said mold and core at sufficient speed to drive the molten metal into the conductor receiving openings and into the end ring recesses in said mold by centrifugal force, and continuing such rotation until the poured metal has congealed.

3. In combination with a cylindrical magnetic core member of an induction motor provided with substantially longitudinally extending, conductor receiving openings therethrough, of a mold comprising end flange portions and cylindrical portions extending beyond the ends of the core, and means for rotating said core and mold.

4. In combination with a cylindrical magnetic core member of an induction motor provided with substantially longitudinally extending, conductor receiving openings therethrough, of a mold comprising end flange portions and cylindrical portions extending beyond the ends of the core, one of said end flange portions being provided with an opening through which molten metal is received for forming conductors in said conductor receiving openings in said core and rings for short-circuiting the conductors at the ends of the core, and means for rotating said core and mold.

5. In combination with a cylindrical magnetic core member of an induction motor provided with substantially longitudinally extending, conductor receiving openings therethrough, of a mold comprising end flange portions, cylindrical portions extending beyond the ends of the core, and means for clamping said end flange portions and said cylindrical portions in place, one of said end flange portions being provided with an opening through which molten metal is received for forming conductors in the conductor receiving openings in said core and rings for short-circuiting the conductors at the ends of the core, and means for rotating said core and mold.

6. The combination with a cylindrical, magnetic core member of an induction motor provided with substantially longitudinally extending, conductor receiving openings therethrough, of a mold comprising end flange portions and a member embracing the outer periphery of said core and extending beyond the ends of the core, and means for rotating said core and mold.

7. The combination with a cylindrical, magnetic core member of an induction motor provided with substantially longitudinally extending, conductor receiving openings therethrough, of a mold comprising end flange portions and a member embracing the outer periphery of said core and extending beyond the ends of the core, one of said flanges being provided with an opening through which molten metal is received for forming conductors in the conductor receiving openings in said core and

rings for short-circuiting the conductors at the ends of the core, and means for rotating said core and mold.

8. The combination with a cylindrical, 5 magnetic core member of an induction motor provided with substantially longitudinally extending, conductor receiving openings therethrough, of a mold comprising a member embracing the outer periphery of 10 said core and extending beyond the ends of the core, end flange portions, and means for clamping said flanges to said member, and means for rotating said core and mold.

9. The combination with a cylindrical, 15 magnetic core member of an induction motor provided with substantially longitudinally extending, conductor receiving openings therethrough, of a mold comprising a member embracing the outer periphery of 20 said core and extending beyond the ends of the core, end flange portions, and means for clamping said flange portions to said member, one of said flange portions being provided with an opening through which 25 molten metal is received for forming conductors in the conductor receiving openings in said core and rings for short-circuiting said conductors at the ends of said core, and means for rotating said core and 30 mold.

10. The combination with a cylindrical, magnetic core member of an induction motor provided with substantially longitudinally extending, conductor receiving open-

ings therethrough, of a mold comprising a 35 member divided along lines substantially parallel to the axis of said core member into a plurality of parts, said parts embracing the outer periphery of said core and extending beyond the ends of the core, 40 end flange portions, and means for clamping said flange portions to said member, and means for rotating said core and said mold.

11. The combination with a cylindrical, 45 magnetic core member of an induction motor provided with substantially longitudinally extending, conductor receiving openings therethrough, of a mold comprising a member divided along lines substantially 50 parallel to the axis of said core member into a plurality of parts, said parts embracing the outer periphery of said core and extending beyond the ends of the core, end flange portions, and means for clamping 55 said flange portions to said member, one of said flange portions being provided with an opening through which molten metal is received for forming conductors in the conductor receiving openings in said 60 core and rings for short-circuiting the conductors at the ends of the core, and means for rotating said core and mold.

In witness whereof, we have hereunto set our hands this 29th day of March 1915.

HENRY G. REIST.  
HOWARD MAXWELL.